

## UNITED STATES PATENT OFFICE

2,171,108

## METHOD OF STABILIZING SILICON ALLOYS

Ernest F. Doom, Niagara Falls, N. Y., assignor to  
 Electro Metallurgical Company, a corporation  
 of West Virginia

No Drawing. Application June 29, 1937,  
 Serial No. 150,938

2 Claims. (Cl. 148—7)

This invention relates to the production of comminuted silicon alloys having improved resistance to surface oxidation and chemical attack.

Powdered or ground silicon alloys find numerous applications in the metallurgical arts. An example of such applications is the use of powdered ferrosilicon as a constituent of the flux coating on welding rods. Used for this purpose, the silicon deoxidizes the deposited metal during welding and also inhibits the loss by oxidation of valuable alloying elements which are normally introduced into the weld metal as constituents of the core or the coating of the rod. The ingredients of many common welding fluxes include certain alkaline constituents, entirely necessary for specific purposes, which tend to react with the silicon, yielding hydrogen as a product of the reaction. Such evolution of gas interferes with the production of a satisfactory coating on the welding rods.

Other common applications of powdered silicon alloys are as a mold wash and as a mold coating. For these purposes the alloy, usually in a finely divided form, is applied to the mold surface on which it functions as an insulating layer for subsequently introduced molten metal, or forms a coating on the surface of the casting depending on the composition and particle size of the powdered alloy. Powdered silicon alloy is readily ignited and when once ignited burns rapidly and almost completely to oxide. For this reason, special precautions must be taken to prevent the destruction of the mold wash and mold coating during pouring of the molten metal.

An object of the present invention is to provide comminuted silicon alloys having improved resistance to surface oxidation and chemical attack, so that difficulties such as those described above may be avoided in the use of these alloys.

The present invention is a method which comprises forming, by a suitable heat treatment, an oxide film on the surface of comminuted silicon alloys. More specifically, a comminuted silicon alloy containing more than 35% silicon is heated in a furnace, in the presence of air or other oxidizing atmosphere, to a temperature below 1000° C. but at least as high as the lowest temperature at which surface oxidation occurs. The lowest useful temperature will be different for alloys having different compositions but, with the exception of the higher silicon alloys, this temperature will usually be between 300° C. and 700° C. The length of the treatment will depend on the particle size of the alloy and the thickness of oxide film desired. Some color change is generally produced on the alloy surfaces, slight in the treatment of certain alloys such as ferrosilicon, but more marked in other silicon alloys.

A preferred method of controlling the rate and extent of surface oxidation, which may proceed

too rapidly when treating large and compact masses, is to heat the powdered metal in small increments or in a thin stream as it passes through a rotating heated cylinder or over a heated surface. The present invention, however, is not limited to these methods of heating.

A specific example of the production of a comminuted silicon alloy having surfaces stabilized in accordance with the present invention is as follows: A charge consisting of 100 grams of a powdered ferrosilicon alloy containing 75% silicon, pulverized to 100 mesh and smaller, was heated in contact with air in a muffle furnace at a temperature of about 1000° C. for a period of one hour. This heat treatment was sufficient to form a thin protective coating of oxide on the surface of each grain of alloy. Tests made on samples of the alloy to determine the amount of gas evolved in alkali media showed that the treated alloy possessed a much slower reaction rate than an untreated ferrosilicon alloy of the same composition.

Equally as good results were obtained from gas evolution tests made on a powdered ferrosilicon alloy containing 50% silicon which had been treated according to a method of the invention at a temperature of 600° C. for a period of one hour.

Comminuted silicon alloys treated in accordance with the present invention are difficult to ignite and therefore are much safer to handle and transport than untreated alloys. Further, powdered silicon alloys having oxidized surfaces are substantially resistant to alkaline and aqueous attack and may be compounded in welding rod coatings containing these media without a substantial evolution of gas.

Although I have described, as an example, the production of powdered ferrosilicon alloys having surfaces substantially resistant to oxidation or chemical attack, it is within the invention to treat, in a similar manner, other powdered or comminuted alloys containing more than 35% silicon.

I claim:

1. A method of preparing a chemically stable unbonded finely comminuted silicon alloy containing more than 35% silicon for use as a constituent of alkaline coating compositions, which comprises forming a thin superficial protective coating of oxide on said comminuted alloy by heating it in an oxidizing atmosphere at a temperature between 300° C. and 1000° C. for a time too short to cause the oxidation of a major part of the alloy.

2. A method as defined in claim 1, wherein the temperature at which the comminuted alloy is heated is between 300° C. and 700° C. and the oxidizing atmosphere is air.

ERNEST F. DOOM. 60